

J. A. SINGMASTER, F. G. BREYER AND E. H. BUNCE.  
PRODUCTION OF METAL OXIDS AND OTHER COMPOUNDS OF METALS.  
APPLICATION FILED JULY 22, 1919.

1,322,143.

Patented Nov. 18, 1919.

3 SHEETS—SHEET 1.



J. A. SINGMASTER, F. G. BREYER AND E. H. BUNCE.  
PRODUCTION OF METAL OXIDS AND OTHER COMPOUNDS OF METALS.  
APPLICATION FILED JULY 22, 1919.

1,322,143.

Patented Nov. 18, 1919.

3 SHEETS—SHEET 2.



Inventors  
Frank G. Breyer  
James A. Singmaster  
Carl H. Bunce  
By their Attorneys  
Pennie, Davis, Marvin & Edmonds.

J. A. SINGMASTER, F. G. BREYER AND E. H. BUNCE.  
PRODUCTION OF METAL OXIDS AND OTHER COMPOUNDS OF METALS.  
APPLICATION FILED JULY 22, 1919.

1,322,143.

Patented Nov. 18, 1919.

3 SHEETS—SHEET 3.



Fig. 7.



Fig. 6.



Inventors  
Frank G. Breyer  
James A. Singmaster  
By their Attorneys  
Carl H. Bulice  
Pennie, Davis, Marnen & Edmunds

# UNITED STATES PATENT OFFICE.

JAMES A. SINGMASTER, OF NEW YORK, N. Y., AND FRANK G. BREYER AND EARL H. BUNCE, OF PALMERTON, PENNSYLVANIA, ASSIGNEES TO THE NEW JERSEY ZINC COMPANY, OF NEW YORK, N. Y., A CORPORATION OF NEW JERSEY.

## PRODUCTION OF METAL OXIDS AND OTHER COMPOUNDS OF METALS.

1,322,143.

Specification of Letters Patent. Patented Nov. 18, 1919.

Application filed July 22, 1919. Serial No. 312,568.

*To all whom it may concern:*

Be it known that we, JAMES A. SINGMASTER, residing at New York city, county and State of New York, FRANK G. BREYER and EARL H. BUNCE, both residing at Palmerton, county of Carbon, State of Pennsylvania, have invented certain new and useful Improvements in the Production of Metal Oxids and other Compounds of Metals (Case F;) and we do hereby declare the following to be a full, clear, and exact description of the invention, such as will enable others skilled in the art to which it appertains to make and use the same.

This invention relates to the production of metal oxids or other compounds of metals volatilized by the Wetherill process, and has for its object the provision of an improved method of producing metal oxids, or other compounds of metals volatilized by the Wetherill process in a continuous operation, as well as the provision of an improved apparatus for carrying out the method of the invention.

Metallic oxids, such, for example, as zinc oxid and leaded zinc oxid, as well as other compounds of metals volatilized by the Wetherill process, such for example, as basic lead sulfate or sublimed lead, have heretofore been more or less extensively produced by the so-called Wetherill process. In speaking of metals volatilized by the Wetherill process, we intend to describe and cover such metals as are volatilizable at the temperatures attainable in the Wetherill process, and for the sake of brevity, we shall hereinafter designate these metals as volatilizable metals. In the case of certain of such metals, the final or desired compound or compounds thereof are the result of a sequence of actions in which the metalliferous materials of the charge are reduced, the reduced metal volatilized and then oxidized or otherwise compounded, while in other cases a metal compound may be directly volatilized, with or without subsequent oxidation or compounding.

By the expression "Wetherill process," as we have used the same herein, is to be understood the furnacing step of the process for producing metal oxids or other compounds of volatilizable metals in which a charge of the metalliferous material mixed with a reducing agent and spread on an

ignited bed of fuel is subjected to a combustion supporting blast or draft and brought to a sufficiently high temperature to reduce the metalliferous materials and volatilize the reduced metal or metals (and (or) to volatilize a metal or a metal compound or compounds) without bringing the charge to a condition where it becomes impervious to the blast or draft, the entire charge being supported on a furnace hearth or grate designed to hold it without letting any considerable part drop through, and the worked-off material being discharged as a clinker or sinter. The "furnacing step" is independent of the subsequent treatment of the laden furnace gases and of the collection of the metal compound or compounds.

As a typical example of the Wetherill process, as heretofore usually practised, we will briefly describe the customary procedure in the commercial production of zinc oxid, including leaded zinc oxid. The furnacing step is generally carried out in a furnace having a broad expanse of horizontal grate or hearth roofed over with an arch, and associated with appropriate instrumentalities for permitting the passage therethrough and into the charge, by either a blast or draft, of a combustion supporting gas. It is customary to first charge upon the furnace grate or hearth a layer of "buckwheat" anthracite coal (which is thereupon ignited usually by the residual heat of the furnace) and by means of a forced blast or draft of air to bring this initial layer of coal to well-developed combustion. Upon this layer of "bed coal" is then charged the customary mixture or "working charge" characteristic of the Wetherill process, that is to say, a mixture of finely divided reducing coal with the finely divided zinkiferous (or zinkiferous and plumbiferous) material, such as zinc silicate, roasted zinc blends, roasted so called "mixed sulfids" of zinc and lead, spelter retort residues, or other reducible zinc-containing or zinc- and lead-containing material at the disposal of the operator. The forced air draft is continued, and, when the familiar flames of greenish tint, known as "zinc candles," begin to make their appearance above the upper surface of the charge, indicating that the reduction and volatilization of the zinc and its oxidation to the

form of fume is well under way, the products of combustion carrying the zinc oxid fume and other volatilized metallic compounds are conveyed through the customary 5 cooling flues, etc., to the bag-room wherein, in a cooled condition, they filter through the bags and pass off into the atmosphere, leaving the fume collected in the interior of the bags, from which it is removed at convenient 10 intervals. The furnace operation is continued until the production of fume therefrom in appreciable quantity ceases, whereupon the residual charge, which is, to a large extent, sintered together, is broken up by long-handled rabbles and pried up and lifted or scraped out through the furnace doors into a receiving pit, or the like, preparatory to the starting of a new operation. The coal or other carbonaceous material 15 of the charge serves the two-fold purpose of furnishing a reducing agent for effecting the reduction of the metalliferous materials of the charge and of furnishing, by combustion, the necessary degree of heat 20 to bring these materials to the reducing temperature characteristic of the process.

As thus ordinarily practised, the above described furnace operation is attended with certain defects interfering with its full efficiency. Prominent among these defects is the inevitable tendency to the formation of blow-holes or craters at various regions of the charge. Working or rabbelling of the charge to break up these blow holes involves 25 considerable labor, and in addition the formation of blow-holes causes waste of fuel and inefficiency in the recovery of values. A further defect of the above described furnace operation is that the forced draft tends 30 to project into the free space above the charge more or less dust, and this dusting is further aggravated by the rabbelling operations. This dust contaminates the fume and damages its color and marketability. These and many 35 of the other defects of the above described furnace operation as heretofore generally practised are overcome to a very remarkable extent by modifying the heretofore customary practice in accordance with the improvements 40 described in the application for Letters Patent of the United States of Frank G. Breyer, James A. Singmaster and Albert E. Hall, Ser. No. 270,179, filed January 8, 1919. These improvements consist in supplying 45 either or both the bed fuel and the working charge to the furnace hearth in the form of briquets. The improved results attendant upon this modification in the prior customary practice are described in detail in 50 the aforementioned application.

In commercial practice, the furnace in which the Wetherill process is carried out has heretofore been generally constructed as a block containing several grate units. 55 Thus, it is customary to build the furnace

or block with four to twelve grate units, each of which may, for example, be about four feet wide and about ten feet long. These grate units may be arranged side by side, or half of the grate units may be arranged side by side and the two halves arranged back to back. The purpose of this arrangement is to get relative continuity of action in the treatment of charges that individually are worked intermittently. Thus, 70 while the operation of the furnace or block may, for practical purposes, be considered more or less continuous, the operation with respect to any individual grate unit is intermittent.

One of us, James A. Singmaster, has described and claimed in U. S. Letters Patent Nos. 1,112,853 and 1,112,854, patented Oct. 6, 1914, a process and apparatus for producing sublimed metallic products by the Wetherill process in which the ignited charge is advanced through a suitable combustion zone in a continuous manner. One of the difficulties encountered in attempting to advance through a combustion zone a charge 80 of finely-divided materials, such as the heretofore customary Wetherill process charge, supported on a movable perforated grate, is that of providing a seal at the sides of the charge. The relative motion between the 85 side walls of the combustion zone and the moving charge provides a very susceptible region for the air blast to break through the charge, and because of this relative movement it is practically impossible to provide 90 an effective seal between the moving charge and the stationary furnace walls with which it directly contacts. In the aforementioned Letters Patent this difficulty is avoided by supporting the charge during its movement 95 through the combustion zone on grate sections so arranged that the moving charge is not in contact with any stationary element, the grate sections themselves being designed 100 to effect the desired seal between the moving 105 and stationary parts.

We have now discovered that very remarkable results are attained, when the Wetherill process is carried out as a continuous operation by advancing an ignited 115 working charge through a suitable combustion zone, by supplying to the moving furnace hearth either or both the layer of bed fuel and the working charge in the form of briquets. The present invention thus contemplates advancing through a suitable combustion zone a working charge containing a briquetted mixture of metalliferous material and a reducing agent spread on an ignited 120 layer of bed fuel, also preferably in the 125 form of briquets, and simultaneously passing a combustion supporting gas into the charge.

In our preferred practice, the working charge, in the form of briquets made up of 130

a mixture of metalliferous materials, such, for example, as zinkiferous, or plumbiferous, or plumbiferous-zinkiferous material, and an appropriate reducing agent, is spread upon a well ignited layer of bed fuel also in the form of briquets, and the entire charge, supported on a perforated furnace hearth, is advanced through a suitable combustion zone or chamber. The fuel briquets may, if desired, contain such a percentage of the metalliferous material as will not interfere with their normal function.

The bed fuel briquets may be prepared by compressing finely divided coal, together with a suitable binder, such, for example, as the concentrated waste sulfite liquor of the sulfite paper pulp industry. Various forms and grades of carbonaceous material are available for the bed fuel briquets. Thus, for example, anthracite coal below the No. 3 buckwheat size, such as No. 4 buckwheat, colliery washing, "dirt" coal, "dust" coal, as well as coke breeze, may be utilized in the production of the bed fuel briquets. The bed fuel briquets are of such size and shape as to materially reduce the resistance to the combustion supporting gas, and nevertheless to supply such a substantially uniform substratum for the support of the superposed working charge as to give free access therethrough and practically equal distribution thereto of the combustion supporting gas. To this end, the bed fuel briquets, as well as the working charge briquets, should be of substantially uniform size, and preferably of such shape that they roll or tumble easily over one another. Thus, we have found the so-called pillow block, egglette, rounded pillow block, over-stuffed pillow, and similar shapes well suited to the purposes of the invention.

While the working charge consisting of a mixture of the metalliferous material and an appropriate reducing agent may be supplied to the ignited layer of bed fuel briquets in an unbriqueted form, we prefer to briquet the working charge because of the many attendant advantages. Furthermore, we wish it to be understood that the metalliferous material may be briqueted alone, without briquetting the reducing agent, or the reducing agent may be briqueted alone without briquetting the metalliferous material or the reducing agent and the metalliferous material may be separately briqueted. However, our preferred practice is to briquet a mixture of the metalliferous material and the reducing agent.

The reducing agent of the working charge may be of any suitable kind, and while we now prefer to employ carbonaceous material as the reducing agent, it will be understood by those skilled in the art that reducing agents other than carbonaceous materials are available for the purposes of the invention.

One of the advantages of employing a briquetted reducing agent in any of the forms hereinbefore described is that it permits the use of carbonaceous materials of cheaper grades and finer mesh, such as anthracite 70 coal of finer mesh than No. 3 buckwheat, colliery washings, dust coal, coke breeze and the like.

The bed fuel briquets and the working charge briquets may be prepared in any 75 appropriate manner. We have found the procedure described in the aforementioned application of Frank G. Breyer, James A. Singmaster and Albert E. Hall, Serial No. 270,179, for preparing similar fuel and 80 working charge briquets well adapted for the purposes of our present invention. This procedure involves generally the steps of mixing the material to be briquetted with a suitable binder, such as concentrated waste 85 sulfite liquor of 30° Baumé, molding the mixture into briquets of the desired size and shape, and drying or baking the briquets at a temperature of approximately 200° C., so as to impart to them the desirable amount of 90 resistance to crumbling and breaking so that they may be freely subjected to the rough handling incident to storing them, conveying them to the furnace, and incident to charging them into the furnace either by hand or 95 otherwise. In the case of the briquetted metalliferous material, it is also desirable that the briquets possess such resistance to crumbling and breaking as to substantially 100 maintain their form during the entire furnacing operation, so that they are for the greater part discharged from the furnace in substantially their original physical form.

The remaining novel features of the invention can be best explained by reference to 105 the accompanying drawings, in which:—

Figure 1 is a sectional elevation of our improved furnace structure; Fig. 2 is a side elevation of the same; Fig. 3 is a top plan of the furnace; Figs. 4, 5 and 6 are sectional 110 views taken on the section lines 4—4, 5—5 and 6—6, respectively; Fig. 7 is a sectional view of the water-cooled leveler for the briquetted working charge, and Fig. 8 is a detail view of the perforated furnace hearth. 115

The furnace illustrated in the drawings has a movable or traveling hearth 10 in the form of a continuous belt or conveyer. The furnace hearth may advantageously be of the general design used in mechanical 120 stokers. As thus constructed, the hearth is made up of a plurality of grate sections secured at their ends to sprocket chains 11. Each grate section is composed of a rigid frame piece having a dove-tailed web on 125 which are strung or keyed the relatively narrow members 12. The members 12 while mechanically contacting with one another permit the passage of the combustion supporting gas therebetween. The spaces be- 130

tween adjacent grate sections and between adjacent members 12 of each grate section provide perforations or small passages uniformly distributed over the entire area of 5 the hearth.

The two sprocket chains 11 coöperate with and are driven by sprocket wheels 13 and 14 secured to shafts 15 and 16, respectively, at opposite ends of the furnace. The shafts 10 15 and 16 are connected through similar worm reduction drives 17 and 18, beveled gears 19 and 20 and worm reduction drives 21 and 22, respectively, to a common shaft 23. The shaft 23 may be driven from any

15 suitable power source, and to this end we have represented a pulley 24, adapted to be operatively connected to the source of power, such, for example, as an electric motor. By 20 this arrangement the shafts 15 and 16, at opposite ends of the furnace, are driven at the same speed, and the furnace hearth 10 is thereby positively driven by the coöperating sprocket wheels at each end of the furnace.

The furnace housing is constructed of 25 fire brick in substantially the usual manner, with a casing of red brick on the outside. The brick work of the furnace structure, and in particular, the arches and skewbacks, are held in position by vertical buckstays 25 30 and transverse tie-rods 26. The buckstays 25 are preferably pivoted at their lower ends to anchor plates 27, preferably embedded in concrete. Relatively heavy coil springs 28 are associated with the tie-rods 26, for forcing 35 coöperating pairs of buckstays on opposite sides of the furnace structure toward one another, thereby maintaining the buckstays firmly pressed against the skewback plates 29.

40 The skewback plates 29 are L-shaped, as will be seen by reference to Figs. 4 and 6 of the drawings, and are arranged to support the skewbacks 30. The furnace arches are supported by the skewbacks 30 in the usual 45 manner, as will be more particularly pointed out hereinafter. It will be observed by reference to Figs. 4 and 6 of the drawings, that the buckstays 25 contact only with the skewback plates 29, and are thus separated 50 by a small space from the side wall of the brick work structure. By this arrangement the tie rods 26 and coöperating springs 28 serve to force each coöperating pair of buckstays firmly against the skewback plates 29,

55 and thus any shrinkage in the brick work structure of the furnace arch, as the furnace dries out, is taken care of and the danger of the arch falling in is practically eliminated. The pivot mounting of the buckstays 25 at 60 their lower ends permits the necessary movement of the buckstays about this pivot to compensate for shrinkage or expansion of the furnace arch.

65 The interior of the furnace housing is divided into a series of chambers by suspended

arches. Thus, an ignition or fuel combustion chamber 31 is provided at the charging end of the furnace by the suspended arches 32 and 33. An ore combustion chamber 34 is provided between the suspended arches 35 and 36. The arches 33 and 35 are suitably spaced in order to accommodate the charging devices for the briqueted working charge, as will be fully described herein-after. The fume-emitting or oxid-making chamber 79 of the furnace is located between the suspended arches 36 and 37.

Three off-takes 38, 39 and 40 are provided for conducting away from the fume-emitting zone the effluent produced therein as the result of the operation. The off-takes 38, 39 and 40 may be connected to separate fume-collecting devices, or may communicate with a common flue and fume-collecting device. The ignition chamber 31 has an off-take 41, and the ore combustion chamber 34 has an offtake 42. The gases passing through the offtakes 41 and 42 may be wasted or subjected to any proper treatment.

90 At the discharge end of the furnace a chamber 43 is provided between the suspended arch 37 and the arch 37'. On one side of the chamber 43 there is an observation door 44, while on the other side there 95 is a sliding door 45. These doors are provided as means of easy access to the rear sprockets 14. Observation doors 46 are provided at appropriate intervals on each side of the furnace opening directly into the 100 combustion chambers or zones thereof.

95 The suspended arches 32, 33, 36 and 37 are held in position in substantially the same manner. Each of these arches is built of a plurality of rectangular fire brick. Rods 47 105 are embedded in these rectangular fire bricks and passing upwardly through the furnace arch and roof are secured in place by being bolted to transverse beams 48. The sector-shaped spaces between the upper surface of these rectangular fire bricks and the curved lower surface of the furnace arch are filled in with fire brick so as to form the desired partition between the various chambers of the furnace.

110 The furnace arch or roof 49 is constructed of fire brick in the usual manner and is supported in position by the skewbacks 30, as will be well understood in the art. A cinder fill 50 may be placed on the top of 120 the arch 49. Along each side wall of the furnace, just above the working surface of the traveling grate 10, carborundum bricks 51 are used to prevent fusion between the charge and the side walls of the furnace.

125 A hopper 52 is arranged at the front or charging end of the furnace for feeding the briqueted bed fuel on to the traveling grate. A gate or charge leveler 53 is associated with the hopper and is adapted to be raised 130

or lowered by means of a wheel 54, and co-operating mechanism. By thus raising or lowering the gate 53, the depth of charge fed on to the traveling grate 10 may be regulated to the desired amount.

5 A hopper 55 is arranged to discharge into the space between the suspended arch 33 and the arch 35. A water-cooled gate or leveler 56 is arranged behind the hopper 55 for leveling the charge fed on to the traveling grate by the hopper. The gate 56, as will be seen by reference to Fig. 7 of the drawings, comprises a hollow shell having transverse baffles 57 for imparting to the cooling medium flowing therethrough a circuitous path. This cooling medium, such, for example, as water, may be supplied to the interior of the hollow shell by an inlet pipe 58, and withdrawn by an outlet pipe 59.

10 The gate 56 is suspended from the top of the furnace structure by vertical rods 60 and may be vertically adjusted with respect to the moving grate by means of the nuts 61.

25 As hereinbefore explained, the drive for the traveling grate is connected so that the grate is driven both from the front and rear through the main power shaft. The return grate is supported on riding bars 62 fastened to the side plates 63 of the furnace.

30 The working floor of the furnace is supported on a suitable foundation 64, preferably elevated so as to facilitate the discharge of the exhaust material from the end of the furnace down an inclined chute 65 into cars

35 or the like.

Above the return or lower portion of the traveling grate 10, and out of contact therewith, is arranged a floor 66, which serves as the bottom wall of the air compartments 40 beneath the upper or working surface of the traveling grate. Four air boxes 67 extend transversely of the furnace structure, at appropriate intervals between the front and rear thereof, and serve to admit the necessary blast of combustion supported gas beneath the perforated grate 10. The space between adjacent air boxes 67 is divided into two compartments by means of the vertical partitions 68. By this arrangement it

50 will be observed that eight air chambers or compartments are provided beneath the perforated traveling grate 10. Wear plates 67' and 68' are preferably mounted on the tops of the air boxes 67 and partitions 68, respectively, to serve as bearing plates for such portions of the traveling grate as contact therewith. The first air compartment at the front or charging end of the furnace is closed on the outside by a sheet metal

60 wall 69, and a similar wall 70 closes the last air compartment at the rear or discharge end of the furnace.

Each of the air boxes 67 extends exteriorly of the furnace at one side, as will be seen

65 by reference to Figs. 2, 3 and 4 of the draw-

ings. Each air box is connected exteriorly of the furnace by a vertical pipe 71 with the main air conduit 72. Each of the pipes 71 is provided with a slide valve 73 for regulating the air supply to its air box. Both 70 of the transverse walls of each air box 67 are provided with twyers or openings 74. A slide damper 75, terminating in a handle 76 exteriorly of the air box, is provided for each series of twyers 74. By moving the 75 handles 76 in or out, the area of the twyers or openings 74 can be adjusted, and in this manner the adjustment of the blast secured. It will be observed that while each air box serves to supply the combustion supporting 80 gas to two air compartments, the amount of gas supplied to each compartment may be regulated by manipulation of the appropriate slide damper 75.

A trough or pan 77 for water is preferably arranged in each of the air compartments, and a pipe 78 may connect with the troughs for conducting water thereto.

In practising the method of our present invention in the furnace illustrated in the 90 accompanying drawings, the fuel briquets are fed in at the front end of the grate through the hopper 52 and the thickness of the bed fuel is regulated by means of the gate 53, which, as hereinbefore explained, 95 may be raised or lowered to any height desired. From this point the fuel briquets travel into the fuel combustion chamber 31 and are there ignited by the high temperature maintained in this chamber. The gases 100 from the fuel combustion chamber are carried off through the stack 41.

At the rear of the fuel combustion chamber, just back of the suspended arch 33, the briquetted working charge is fed on to the 105 ignited fuel briquets through the hopper 55. The depth of the briquetted working charge is regulated by the gate 56, which may be set at any desired height. As previously explained, this gate is cooled by means of 110 circulating water. The briquetted working charge thus spread on the ignited fuel briquets is advanced into what we have called the ore combustion chamber 34, in which the charge is brought up to the reducing temperature. The stack 42 is provided so that, if desirable, the effluent made in this chamber may be recovered separately from that produced in the main oxid-making chamber 79.

115 The briquetted charge now passes under the suspended arch 36 into the main effluent of fume emitting chamber 79, in which the active reduction of the charge takes place. The blow or blast in this chamber is so regulated that complete reduction takes place by the time the charge has traveled to the rear of the chamber. From the exhaust chamber the three off-takes 38, 39 and 40 conduct the effluent to the flue system and fume collect- 125

ing devices, as will be well understood in the art. Each of the off-takes 42, 38, 39 and 40, is provided with a slide damper 42', 38', 39' and 40' respectively, for regulating the flow 5 of the effluent so as to help control the temperature at all points of the chamber 79. A trailing door or gate 80 is operatively mounted on the suspended arch 37 for preventing the passage underneath the arch 10 and into the chamber 79 of currents or drafts of air.

From the fume emitting chamber 79, the worked-off briquets pass underneath the suspended arch 37 into the rear chamber 43. 15 This chamber is also provided with a stack 82, for balancing the draft between the rear chambers and the fume emitting chamber. As the grate sections pass over the rear sprockets 14, the worked-off charge, consisting of a light coal clinker and worked-off briquets, is discharged on to the chute 65 and thence into the receiving hoppers (not shown). A pendant door or gate 81 is pivoted to the arch 37' and serves to maintain 20 the residue discharge opening of the chamber 43 normally closed. When a certain amount of residue banks up against this door 81 it swings open to permit the discharge of the residue down the chute 65.

30 The traveling furnace hearth moves at a very slow speed, a few feet per hour. The speed of the hearth will be determined by the dimensions of the fume-emitting zone, the character and quantity of metalliferous 35 material charged and other considerations, which will be understood by those skilled in the art. In producing zinc oxid in accordance with the invention, we have found a temperature of approximately 1100 to 1250° 40 C. well suited for the fume-emitting or oxid-making chamber or zone, when using the well known Franklin furnace zinc oxid ores, and at this temperature the briquetted working charge can ordinarily be satisfactorily 45 worked-off or depleted of its zinkiferous content in from two and one-half to three and one-half hours, when operating with a furnace whose oxid-making chamber 79 is about eighteen feet in length and with a 50 grate speed of about seven feet per hour.

In the customary commercial practice of the Wetherill process, the total carbonaceous material in the entire charge, including the bed fuel and the working charge mixture, is 55 several times greater than the theoretical amount required to reduce the compounds of the volatilizable metals in the charge. It has heretofore been the general practice to place the greater proportion of the total carbonaceous material of the charge in the working charge mixture. For example, in the production of zinc oxid, when operating with the well known Franklin furnace zinc oxid ores, it is customary to place from about 60 65 15 to 25 per cent. of the total carbonaceous

material of the entire charge in the bed fuel, while the remaining 85 to 75 per cent. of the total carbonaceous material is mixed with the ore to form the working charge. In general terms, the layer of bed fuel is approximately one inch in depth or thickness, while the working charge mixture is spread over the ignited bed fuel in a layer from about five to seven inches in depth or thickness. 70

A very decided improvement in the efficiency of the Wetherill process can be secured by placing the greater proportion of the total fuel of the charge in the form of briquets in the bed fuel, rather than in the working charge as has heretofore been customary. This improvement in the heretofore customary practice of the Wetherill process is described and claimed in an application for Letters Patent of the United States of Frank G. Breyer, Albert E. Hall and George R. Waltz, Serial No. 310,440, filed July 12, 1919. When a very considerable proportion of the carbonaceous or other combustible material of the entire charge is thus withdrawn from the working charge and placed in the bed fuel in the form of briquets, the residual charge consists of a relatively thin clinkered ash, resulting from the combustion of the bed fuel briquets, and the worked-off metalliferous material. When the metalliferous material has been briquetted and spread on the ignited bed fuel briquets, the worked-off ore briquets are discharged in substantially their original physical form, so that the worked-off briquets may be readily separated from the clinkered ash of the bed fuel briquets. Furthermore, in view of the fact that the working charge briquets contain only a relatively small amount of the total carbonaceous material of the charge, the resulting amount of ash in the worked-off metalliferous or ore briquets is relatively small, and such worked-off briquets may on this account be very advantageously employed in subsequent smelting operations for the recovery therefrom of further metallic values, as will be more fully described hereinafter. Accordingly, in view of the attendant advantages, it is our preferred practice in carrying out the present invention to place the greater part of the total combustible material of the entire charge in the bed fuel briquets, and we have secured excellent results by placing from about 75 to about 85% of the total carbonaceous or combustible material of the entire charge in the bed fuel briquets. 100

As a typical instance of the practice of the invention, we will briefly describe, in connection with the production of zinc oxid, a particular operation in which both fuel briquets and a briquetted working charge were used. Eight-five (85) per cent. of the total coal of the entire charge was carried in the 105 110 115 120 125 130

bed fuel briquets, leaving fifteen (15) per cent. of the total coal for mixture with the zinkiferous material in the working charge. The fuel briquets were made up of washed 5 coal with three (3) per cent. concentrated waste sulfite liquor binder. The briquetted working charge consisted of a mixture of ninety (90) per cent. zinkiferous material and ten (10) per cent. washed dust coal, to 10 which three (3) per cent. waste sulfite liquor was added as a binder. Both the ore and fuel briquets were of the rounded pillow block type.

The levelers or gates 53 and 56 of the accompanying drawings were set to deliver a 15 layer of bed fuel six inches deep and a three inch layer of the briquetted working charge.

In the foregoing operation we secured 20 very satisfactory results by holding the fuel ignition chamber 31 at the minimum temperature for uniform ignition, that is, from about 800° to 950° C.; the ore ignition chamber 34 at a temperature where a light zinc flame is visible, for example, from 1000° to 25 1050° C., and the oxid-making chamber 79, at a uniform temperature of from 1100° to 1250° C., since at this temperature reduction is active, and with the usual working mixtures only incipient fusion of the briquetted 30 working charge takes place, so that none of the zinc is trapped into the slag.

The oxid made in accordance with the foregoing operation is decidedly superior to that made from charges of the same ore on the customary oxid furnace blocks. It is 35 particularly free from any grit or specks and very bright. The recoveries of zinc from the working charge are remarkably high, and we have found by the practice of our invention, that it is possible to secure recoveries 40 better than ninety per cent. as indicated by the clinker analysis.

No bars or rakes need be used, nor need 45 the charge be disturbed in any manner in practising the method of our present invention. The only labor necessary consists in feeding the briquets to the furnace and carting away the clinker and worked-off briquets discharged into the hoppers or cars provided 50 therefor. There is, furthermore, no blow-hole trouble, and no sticking of the charge to the side walls and no loss of blow at the side walls. The briquets feed uniformly and the ignition of both fuel and working charge 55 briquets is very uniform. The clinker, consisting of a relatively thin layer of coal ash and burned-out briquets, discharges readily and no labor is attendant upon the discharging operation.

60 When, as in the preferred embodiment of the invention, the metalliferous material of the working charge is supplied to the furnace hearth in the form of briquets, the worked-off ore briquets retain for the most 65 part their original shape with only incipient

fusion. Some of the working charge briquets will almost inevitably become broken or crushed in the preliminary handling and furnacing operation, but these briquets for the greater part retain their original physical form. After the furnacing operation, 70 these briquets are remarkably hard and almost coke-like in their physical characteristics, and are readily separated from the clinkered coal ash of the bed fuel briquets. 75

This capability of readily separating the worked-off metalliferous or ore briquets from the ash of the fuel briquets is of especial advantage when the worked-off 80 metalliferous briquets are to be subjected to further treatment for the recovery of valuable metals not volatilizable by the Weth-erill process. Where the working charge

briquets consist of a mixture of metalliferous material and carbonaceous reducing 85 agent, the worked-off briquets will contain, in addition to the worked-off metalliferous material, the ash from the consumed carbonaceous reducing agent as well as the un- 90 consumed portion of the reducing agent. 90

The ash is composed principally of silicia and alumina, and is generally objectionable in any subsequent treatment of the worked-off metalliferous briquets. Thus for 95 example, in those instances in which the un-worked-off metalliferous briquets are smelted in a blast furnace for the production of spiegeleisen a certain amount of fluxing agents is necessary for slagging off the ash present in the worked-off metalliferous briquets, and when this amount of ash is relatively large an objectionably large amount of fluxing agent is required, with the resultant production of an objectionably large 100 amount of slag.

By placing approximately 105 85% of the total carbonaceous material of the entire charge in the bed fuel briquets, the main bulk, for example, around 85 per cent. of the ash of the total carbonaceous 110 material of the charge is in the clinker resulting from the combustion of the bed fuel briquets, and the worked-off metalliferous briquets are consequently contaminated with only a relatively small amount of ash. On 115 account of this relatively slight ash contamination of the worked-off metalliferous briquets, as well as on account of their physical properties, these briquets are peculiarly well adapted for subsequent treatment in blast furnaces.

In addition to retaining their 120 original form, these briquets are moreover of a porous character, due to the removal of the volatilizable metals therefrom, and this porous property of the worked-off briquets is also of advantage in their subsequent 125 treatment.

While we have hereinbefore specifically described the invention by reference to the production of zinc oxid, including leaded zinc oxid, we wish it to be understood that 130

the invention is applicable to the production of other metal compounds of the volatilizable metals. In particular, we contemplate the production of basic lead sulfate or sublimed lead by the method of the invention. In general, the procedure for the production of sublimed lead is substantially the same as hereinbefore described, substituting, of course, an appropriate plumbiferous material for the zinkiferous material. Thus, for example, the bed fuel is deposited on the traveling hearth of the furnace in the manner hereinbefore described and in accordance with our preferred practice contains in the form of briquets the bulk or greater proportion of the total carbonaceous or other combustible material of the entire charge. The working charge consists of a mixture of finely divided galena or native lead sulfid and carbonaceous material preferably briqueted as hereinbefore described. The working charge is spread on the advancing and ignited layer of bed fuel briquets and upon reaching the reaction temperature, the lead sulfid is reduced and (or) volatilized and subsequently oxidized to lead sulfate and lead oxid thus forming the so-called basic lead sulfate.

The effluent containing the sublimed lead is withdrawn from the furnace and the metallic product collected in any appropriate manner. The worked-off plumbiferous briquets containing as they do a relatively small amount of contaminating ash may be advantageously subjected to any appropriate subsequent treatment for the recovery of the non-volatile metals of the original metalliferous material. As the source of plumbiferous material, we may use a high grade of native lead sulfid suitably crushed and jigged to free it from accompanying gangue material, or we may use lead sulfid concentrates, such as flotation concentrates, or other appropriate plumbiferous-containing material, with proper additions of sulfur in the form of pyrite, galena, brimstone or other suitable sulfur-carrying agents, whenever there is a lack of sulfur in the charge to properly sulfate the fume.

A very accurate and uniform control of the temperature throughout the entire furnace, and hence during the entire furnacing operation of the charge, is secured by the practice of the invention. Thus, the temperature of the various chambers or zones of the furnace can be accurately regulated and controlled by appropriately adjusting the slide dampers 73 of the various air compartments, and the desired operating temperatures are easily maintained throughout the entire furnace. This uniformity of the temperature conditions is attended by practically uniform working conditions of the desired character throughout the furnace, and results in the production of a uniform

product of improved quality, as well as in increased output. Thus, by the practice of the invention, we have been able to secure recoveries better than ninety (90) per cent. of the volatilizable metals of the charge, as indicated by the clinker analyses. The furnacing operation is substantially automatic, and requires only casual attention, thereby effecting a great saving in labor over that required in the operation of the present day types of oxid furnaces. The combustion of the bed fuel is substantially complete, so that practically the full calorific value of the fuel is effectively utilized, thereby enabling a saving in the amount of fuel required as compared with that necessary in working with the heretofore customary types of oxid furnaces. The worked-off briquets are, in our preferred practice, only slightly contaminated with ash and the like, and on this account, as well as on account of their physical form and properties these worked-off briquets are well adapted for subsequent smelting operations.

We claim:—

1. The process of producing metal oxids or other compounds of metals volatilized by the Wetherill process which comprises advancing through a suitable combustion zone a working charge containing a briqueted mixture of metalliferous material and a reducing agent spread on an ignited layer of bed fuel in the form of briquets and simultaneously passing a combustion supporting gas into the charge, and removing the resulting effluent; substantially as described. 90

2. The process of producing metal oxids or other compounds of metals volatilized by the Wetherill process which comprises advancing through a suitable combustion zone a working charge containing a mixture of briqueted metalliferous material and a reducing agent spread on an ignited layer of bed fuel in the form of briquets and simultaneously passing a combustion supporting gas into the charge, and removing the resulting effluent; substantially as described. 95

3. The process of producing metal oxids or other compounds of metals volatilized by the Wetherill process which comprises advancing through a suitable combustion zone a working charge containing briqueted metalliferous material spread on an ignited layer of bed fuel in the form of briquets and simultaneously passing a combustion supporting gas into the charge, and removing the resulting effluent; substantially as described. 100

4. The process of producing metal oxids or other compounds of metals volatilized by the Wetherill process which comprises advancing through a suitable combustion zone a working charge containing a mixture of metalliferous material and a briqueted reducing agent spread on an ignited layer 115 120 125 130

- of bed fuel in the form of briquets and simultaneously passing a combustion supporting gas into the charge, and removing the resulting effluent; substantially as described.
5. The process of producing metal oxids or other compounds of metals volatilized by the Wetherill process which comprises advancing through a suitable combustion zone 10 a working charge containing a mixture of metalliferous material and a reducing agent spread on an ignited layer of bed fuel in the form of briquets and simultaneously passing a combustion supporting gas into the charge, and removing the resulting effluent; substantially as described.
6. The process of producing metal oxids or other compounds of metals volatilized by the Wetherill process which comprises advancing through a suitable combustion zone 20 a working charge containing metalliferous material spread on an ignited layer of bed fuel in the form of briquets and simultaneously passing a combustion supporting gas into the charge, and removing the resulting effluent; substantially as described.
7. The process of producing metal oxids or other compounds of metals volatilized by the Wetherill process which comprises advancing through a suitable combustion zone 30 a working charge containing a briqueted mixture of metalliferous material and a reducing agent spread on an ignited layer of bed fuel and simultaneously passing a combustion supporting gas into the charge, and removing the resulting effluent; substantially as described.
8. The process of producing metal oxids or other compounds of metals volatilized by the Wetherill process which comprises advancing through a suitable combustion zone 40 a working charge containing a mixture of briqueted metalliferous material and a reducing agent spread on an ignited layer of bed fuel and simultaneously passing a combustion supporting gas into the charge, and removing the resulting effluent; substantially as described.
9. The process of producing metal oxids or other compounds of metals volatilized by the Wetherill process which comprises advancing through a suitable combustion zone 50 a working charge containing briqueted metalliferous material spread on an ignited layer of bed fuel and simultaneously passing a combustion supporting gas into the charge, and removing the resulting effluent; substantially as described.
10. The process of producing metal oxids or other compounds of metals volatilized by the Wetherill process which comprises depositing upon a perforated hearth a layer 60 of bed fuel in the form of briquets, igniting said layer of briquets, spreading thereon a working charge containing a briqueted mix- 65
- ture of metalliferous material and a reducing agent, advancing said hearth and the charge supported thereon through a combustion zone and simultaneously passing a combustion supporting gas into the charge, 70 and removing the resulting effluent; substantially as described.
11. The process of producing metal oxids or other compounds of metals volatilized by the Wetherill process which comprises de- 75 positing upon a perforated hearth a layer of bed fuel in the form of briquets, igniting said layer of briquets, spreading thereon a working charge containing a mixture of briqueted metalliferous material and a re- 80 ducing agent, advancing said hearth and the charge supported thereon through a combustion zone and simultaneously passing a combustion supporting gas into the charge, 85 and removing the resulting effluent; sub- stantially as described.
12. The process of producing metal oxids or other compounds of metals volatilized by the Wetherill process which comprises de- 90 positing upon a perforated hearth a layer of bed fuel in the form of briquets, igniting said layer of briquets, spreading thereon a working charge containing briqueted metalliferous material, advancing said hearth and the charge supported thereon through a 95 combustion zone and simultaneously passing a combustion supporting gas into the charge, and removing the resulting effluent; sub- stantially as described.
13. The process of producing metal oxids 100 or other compounds of metal volatilized by the Wetherill process which comprises de- positing upon a perforated hearth a layer of bed fuel in the form of briquets, igniting said layer of briquets, spreading thereon a 105 working charge containing a mixture of metalliferous material and a briqueted re- ducing agent, advancing said hearth and the charge supported thereon through a 110 combustion zone and simultaneously passing a combustion supporting gas into the charge, and removing the resulting effluent; sub- stantially as described.
14. The process of producing metal oxids 115 or other compounds of metals volatilized by the Wetherill process which comprises de- positing upon a perforated hearth a layer of bed fuel in the form of briquets, igniting said layer of briquets, spreading thereon a working charge containing a mixture of 120 metalliferous material and a reducing agent, advancing said hearth and the charge sup- ported thereon through a combustion zone and simultaneously passing a combustion 125 supporting gas into the charge, and remov- ing the resulting effluent; substantially as described.
15. The process of producing metal oxids or other compounds of metals volatilized by the Wetherill process which comprises de- 130

- positing upon a perforated hearth a layer of bed fuel in the form of briquets, igniting said layer of briquets, spreading thereon a working charge containing metalliferous material, advancing said hearth and the charge supported thereon through a combustion zone and simultaneously passing a combustion supporting gas into the charge, and removing the resulting effluent; substantially as described.
16. The process of producing metal oxids or other compounds of metals volatilized by the Wetherill process which comprises depositing upon a perforated hearth a layer of bed fuel, igniting said layer of bed fuel, spreading thereon a working charge containing a briqueted mixture of metalliferous material and a reducing agent, advancing said hearth and the charge supported thereon through a combustion zone and simultaneously passing a combustion supporting gas into the charge, and removing the resulting effluent; substantially as described.
17. The process of producing metal oxids or other compounds of metals volatilized by the Wetherill process which comprises depositing upon a perforated hearth a layer of bed fuel, igniting said layer of bed fuel, spreading thereon a working charge containing a mixture of briqueted metalliferous material and a reducing agent, advancing said hearth and the charge supported thereon through a combustion zone and simultaneously passing a combustion supporting gas into the charge, and removing the resulting effluent; substantially as described.
18. The process of producing metal oxids or other compounds of metals volatilized by the Wetherill process which comprises depositing upon a perforated hearth a layer of bed fuel, igniting said layer of bed fuel, spreading thereon a working charge containing briqueted metalliferous material, advancing said hearth and the charge supported thereon through a combustion zone and simultaneously passing a combustion supporting gas into the charge, and removing the resulting effluent; substantially as described.
19. The process of producing metal oxids or other compounds of metals volatilized by the Wetherill process which comprises depositing upon a furnace hearth a layer of bed fuel containing the greater part of the total combustible material of the entire charge in the form of briquets, igniting said layer of bed fuel briquets, spreading thereon a working charge containing a briqueted mixture of metalliferous material and a reducing agent, advancing said hearth and the charge supported thereon through a combustion zone and simultaneously passing a combustion supporting gas into the charge, and removing the resulting effluent; substantially as described.
20. The process of producing metal oxids or other compounds of metals volatilized by the Wetherill process which comprises depositing upon a furnace hearth a layer of bed fuel containing the greater part of the total combustible material of the entire charge in the form of briquets, igniting said layer of bed fuel briquets, spreading thereon a working charge containing a mixture of briqueted metalliferous material and a reducing agent, advancing said hearth and the charge supported thereon through a combustion zone and simultaneously passing a combustion supporting gas into the charge, and removing the resulting effluent; substantially as described.
21. The process of producing metal oxids or other compounds of metals volatilized by the Wetherill process which comprises depositing upon a furnace hearth a layer of bed fuel containing the greater part of the total combustible material of the entire charge in the form of briquets, igniting said layer of bed fuel briquets, spreading thereon a working charge containing briqueted metalliferous material, advancing said hearth and the charge supported thereon through a combustion zone and simultaneously passing a combustion supporting gas into the charge, and removing the resulting effluent; substantially as described.
22. The process of producing metal oxids or other compounds of metals volatilized by the Wetherill process which comprises depositing upon a furnace hearth a layer of bed fuel containing the greater part of the total combustible material of the entire charge in the form of briquets, igniting said layer of bed fuel briquets, spreading thereon a working charge containing a mixture of metalliferous material and a briqueted reducing agent, advancing said hearth and the charge supported thereon through a combustion zone and simultaneously passing a combustion supporting gas into the charge, and removing the resulting effluent; substantially as described.
23. The process of producing metal oxids or other compounds of metals volatilized by the Wetherill process which comprises depositing upon a furnace hearth a layer of bed fuel containing the greater part of the total combustible material of the entire charge in the form of briquets, igniting said layer of bed fuel briquets, spreading thereon a working charge mixture containing metalliferous material and a reducing agent, advancing said hearth and the charge supported thereon through a combustion zone and simultaneously passing a combustion supporting gas into the charge, and removing the resulting effluent; substantially as described.
24. The process of producing metal oxids or other compounds of metals volatilized by

the Wetherill process which comprises depositing upon a furnace hearth a layer of bed fuel containing the greater part of the total combustible material of the entire 5 charge in the form of briquets, igniting said layer of bed fuel briquets, spreading thereon a working charge containing metalliferous material, advancing said hearth and the charge supported thereon through a combustion zone and simultaneously passing a combustion supporting gas into the charge, and removing the resulting effluent; substantially as described.

25. The method of producing sublimed lead by the Wetherill process which comprises advancing through a suitable combustion zone a working charge containing a briquetted mixture of plumbiferous material and a reducing agent spread on an ignited 15 layer of bed fuel in the form of briquets and simultaneously passing a combustion supporting gas into the charge, and removing the resulting effluent; substantially as described.

25. The method of producing sublimed lead by the Wetherill process which comprises advancing through a suitable combustion zone a working charge containing a mixture of briquetted plumbiferous material and 30 a reducing agent spread on an ignited layer of bed fuel in the form of briquets and simultaneously passing a combustion supporting gas into the charge, and removing the resulting effluent; substantially as described.

35. The method of producing sublimed lead by the Wetherill process which comprises advancing through a suitable combustion zone a working charge containing briquetted plumbiferous material spread on an 40 ignited layer of bed fuel in the form of briquets and simultaneously passing a combustion supporting gas into the charge, and removing the resulting effluent; substantially as described.

45. The method of producing sublimed lead by the Wetherill process which comprises advancing through a suitable combustion zone a working charge containing a mixture of plumbiferous material and a 50 briquetted reducing agent spread on an ignited layer of bed fuel in the form of briquets and simultaneously passing a combustion supporting gas into the charge, and removing the resulting effluent; substantially as described.

55. The method of producing sublimed lead by the Wetherill process which comprises advancing through a suitable combustion zone a working charge containing a 60 mixture of plumbiferous material and a reducing agent spread on an ignited layer of bed fuel in the form of briquets and simultaneously passing a combustion supporting gas into the charge, and removing the resulting effluent; substantially as described.

30. The method of producing sublimed lead by the Wetherill process which comprises advancing through a suitable combustion zone a working charge containing plumbiferous material spread on an ignited 70 layer of bed fuel in the form of briquets and simultaneously passing a combustion supporting gas into the charge, and removing the resulting effluent; substantially as described. 75

31. The method of producing sublimed lead by the Wetherill process which comprises advancing through a suitable combustion zone a working charge containing a briquetted mixture of plumbiferous material 80 and a reducing agent spread on an ignited layer of bed fuel and simultaneously passing a combustion supporting gas into the charge, and removing the resulting effluent; substantially as described. 85

32. The method of producing sublimed lead by the Wetherill process which comprises advancing through a suitable combustion zone a working charge containing a mixture of briquetted plumbiferous material and 90 a reducing agent spread on an ignited layer of bed fuel and simultaneously passing a combustion supporting gas into the charge, and removing the resulting effluent; substantially as described. 95

33. The method of producing sublimed lead by the Wetherill process which comprises advancing through a suitable combustion zone a working charge containing briquetted plumbiferous material spread on an 100 ignited layer of bed fuel and simultaneously passing a combustion supporting gas into the charge, and removing the resulting effluent; substantially as described.

34. The method of producing sublimed lead by the Wetherill process which comprises depositing upon a perforated hearth a layer of bed fuel in the form of briquets, igniting said layer of briquets, spreading thereon a working charge containing a briquetted mixture of plumbiferous material and a reducing agent, advancing said hearth and the charge supported thereon through a combustion zone and simultaneously passing a combustion supporting gas into the charge, 115 and removing the resulting effluent; substantially as described. 110

35. The method of producing sublimed lead by the Wetherill process which comprises depositing upon a perforated hearth a 120 layer of bed fuel in the form of briquets, igniting said layer of briquets, spreading thereon a working charge containing a mixture of briquetted plumbiferous material and a reducing agent, advancing said hearth and the charge supported thereon through a combustion zone and simultaneously passing a combustion supporting gas into the charge, and removing the resulting effluent; substantially as described. 125

65. The method of producing sublimed lead by the Wetherill process which comprises depositing upon a perforated hearth a 130 layer of bed fuel in the form of briquets, igniting said layer of briquets, spreading thereon a working charge containing a mixture of briquetted plumbiferous material and a reducing agent, advancing said hearth and the charge supported thereon through a combustion zone and simultaneously passing a combustion supporting gas into the charge, and removing the resulting effluent; substantially as described.

36. The method of producing sublimed lead by the Wetherill process which comprises depositing upon a perforated hearth a layer of bed fuel in the form of briquets, 5 igniting said layer of briquets, spreading thereon a working charge containing briqueted plumbiferous material, advancing said hearth and the charge supported thereon through a combustion zone and simultaneously 10 passing a combustion supporting gas into the charge, and removing the resulting effluent; substantially as described.

37. The method of producing sublimed lead by the Wetherill process which comprises depositing upon a perforated hearth a layer of bed fuel in the form of briquets, 15 igniting said layer of briquets, spreading thereon a working charge containing a mixture of plumbiferous material and a briqueted reducing agent, advancing said hearth and the charge supported thereon through a combustion zone and simultaneously 20 passing a combustion supporting gas into the charge, and removing the resulting effluent; substantially as described.

38. The method of producing sublimed lead by the Wetherill process which comprises depositing upon a perforated hearth a layer of bed fuel in the form of briquets, 30 igniting said layer of briquets, spreading thereon a working charge containing a mixture of plumbiferous material and a reducing agent, advancing said hearth and the charge supported thereon through a combustion 35 zone and simultaneously passing a combustion supporting gas into the charge, and removing the resulting effluent; substantially as described.

39. The method of producing sublimed 40 lead by the Wetherill process which comprises depositing upon a perforated hearth a layer of bed fuel in the form of briquets, igniting said layer of briquets, spreading thereon a working charge containing plumbiferous material, advancing said hearth 45 and the charge supported thereon through a combustion zone and simultaneously passing a combustion supporting gas into the charge, and removing the resulting effluent; substantially 50 as described.

40. The method of producing sublimed lead by the Wetherill process which comprises depositing upon a perforated hearth a layer of bed fuel, igniting said layer of 55 bed fuel, spreading thereon a working charge containing a briqueted mixture of plumbiferous material and a reducing agent, advancing said hearth and the charge supported thereon through a combustion 60 zone and simultaneously passing a combustion supporting gas into the charge, and removing the resulting effluent; substantially as described.

41. The method of producing sublimed 65 lead by the Wetherill process which com-

prises depositing upon a perforated hearth a layer of bed fuel, igniting said layer of bed fuel, spreading thereon a working charge containing a mixture of briqueted plumbiferous material and a reducing agent, advancing said hearth and the charge supported thereon through a combustion zone and simultaneously passing a combustion supporting gas into the charge, and removing the resulting effluent; substantially as described.

42. The method of producing sublimed lead by the Wetherill process which comprises depositing upon a perforated hearth a layer of bed fuel, igniting said layer of 80 bed fuel, spreading thereon a working charge containing briqueted plumbiferous material, advancing said hearth and the charge supported thereon through a combustion zone and simultaneously passing a 85 combustion supporting gas into the charge, and removing the resulting effluent; substantially as described.

43. The method of producing sublimed lead by the Wetherill process which comprises depositing upon a furnace hearth a layer of bed fuel containing the greater part 90 of the total combustible material of the entire charge in the form of briquets, igniting said layer of bed fuel briquets, spreading thereon a working charge containing a mixture of briqueted plumbiferous material and a reducing agent, advancing said hearth and the charge supported thereon through a combustion zone and simultaneously passing a 95 combustion supporting gas into the charge, and removing the resulting effluent; substantially as described.

44. The method of producing sublimed lead by the Wetherill process which comprises depositing upon a furnace hearth a layer of bed fuel containing the greater part 105 of the total combustible material of the entire charge in the form of briquets, igniting said layer of bed fuel briquets, spreading thereon a working charge containing a mixture of briqueted plumbiferous material and a reducing agent, advancing said hearth and the charge supported thereon through a combustion zone and simultaneously passing a 110 combustion supporting gas into the charge, and removing the resulting effluent; substantially as described.

45. The method of producing sublimed lead by the Wetherill process which comprises depositing upon a furnace hearth a layer of bed fuel containing the greater part 120 of the total combustible material of the entire charge in the form of briquets, igniting said layer of bed fuel briquets, spreading thereon a working charge containing briqueted plumbiferous material, advancing said hearth and the charge supported thereon through a combustion zone and simultaneously passing a 125 combustion supporting gas into the charge, and removing the resulting effluent; substantially as described.

gas in to the charge, and removing the resulting effluent; substantially as described.

46. The method of producing sublimed lead by the Wetherill process which comprises depositing upon a furnace hearth a layer of bed fuel containing the greater part of the total combustible material of the entire charge in the form of briquets, igniting said layer of bed fuel briquets, spreading thereon a working charge containing a mixture of plumbiferous material and a briquetted reducing agent, advancing said hearth and the charge supported thereon through a combustion zone and simultaneously passing a combustion supporting gas into the charge, and removing the resulting effluent; substantially as described.

47. The method of producing sublimed lead by the Wetherill process which comprises depositing upon a furnace hearth a layer of bed fuel containing the greater part of the total combustible material of the entire charge in the form of briquets, igniting said layer of bed fuel briquets, spreading thereon a working charge mixture containing plumbiferous material and a reducing agent, advancing said hearth and the charge supported thereon through a combustion zone and simultaneously passing a combustion supporting gas into the charge, and removing the resulting effluent; substantially as described.

48. The method of producing sublimed lead by the Wetherill process which comprises depositing upon a furnace hearth a layer of bed fuel containing the greater part of the total combustible material of the entire charge in the form of briquets, igniting said layer of bed fuel briquets, spreading thereon a working charge containing plumbiferous material, advancing said hearth and the charge supported thereon through a combustion zone and simultaneously passing a combustion supporting gas into the charge, and removing the resulting effluent; substantially as described.

49. A metallurgical furnace for producing metal oxids or other compounds of metals volatilized by the Wetherill process comprising a combustion chamber, a traveling perforated hearth operatively arranged to support and advance through said chamber a charge containing briquetted material, said briquetted material contacting with the side walls of said chamber and thereby preventing any loss of blow between the advancing charge and the side walls of the chamber; means for depositing a layer of bed fuel on the traveling hearth, means whereby said layer of bed fuel is ignited, means for spreading a working charge on the ignited layer of bed fuel, means for removing the effluent from said combustion

chamber, and means for passing a combustion supporting gas through the perforations of said hearth and into the charge supported thereon.

50. A metallurgical furnace for producing metal oxids or other compounds of metals volatilized by the Wetherill process comprising a combustion chamber, a continuous traveling perforated hearth operatively arranged to support and advance through said chamber a working charge, means for depositing a layer of bed fuel in the form of briquets on the traveling hearth, means whereby said layer of briquets is ignited, means for spreading a working charge containing briquetted material on the ignited layer of bed fuel, the aforesaid briquets of the charge contacting with the side walls of said chamber and thereby preventing any loss of blow between the advancing charge and the side walls of the chamber, means for removing the effluent from said chamber, and means for passing a combustion supporting gas through the perforations of said hearth and into the charge supported thereon.

51. A metallurgical apparatus comprising a combustion chamber, a traveling perforated hearth operatively arranged to support and advance through said chamber a working charge, means for supplying a charge containing briquetted material to said traveling hearth whereby said briquetted material forms an operative seal between the stationary side walls of said chamber and the advancing charge, and means for passing a combustion supporting gas through the perforations of said hearth and into the charge supported thereon.

52. In a process for volatilizing and oxidizing metal values involving the blowing of air into a continuously advancing bed containing the metal bearing material and combustible material under conditions which will leave the worked-off charge as a clinker, and which will produce a volatile fume, the step of supplying at least part of the charge in the form of briquets; substantially as described.

53. In a process for producing sublimed lead involving the blowing of air into a continuously advancing bed containing the metal-bearing material and combustible material under conditions which will leave the worked-off charge as a clinker and which will produce a volatile fume, the step of supplying at least part of the charge in the form of briquets; substantially as described.

In testimony whereof we affix our signatures.

JAMES A. SINGMASTER.  
FRANK G. BREYER.  
EARL H. BUNCE.